

May 11, 1948.

A. H. WARTH ET AL

2,441,173

CAP

Filed Dec. 28, 1942



*Fig. 2.*



Inventors:

Albin H. Warth, Jr.

Paul Grabus, Jr.,

By *Cushman, Daley & Teague* Attorneys.

## UNITED STATES PATENT OFFICE

2,441,173

## CAP

Albin H. Warth and Paul Grabus, Jr., Baltimore,  
Md., assignors to Crown Cork & Seal Company,  
Inc., Baltimore, Md., a corporation of New York

Application December 28, 1942, Serial No. 470,382

2 Claims. (Cl. 215—40)

1

This invention relates to caps particularly of the crown or crimped skirt type but also to lug, screw and pressed-on closures.

The primary object of the invention is to provide a cap having a cushion liner of compressed or suitably densified cellulosic material in lieu of the customary and now difficultly obtainable cork liner and coated on at least its exposed face and preferably on both faces with a thermoplastic coextensive sealing film. This film has the effect of (1) preventing penetration of liquids and gases into the liner, (2) affording a tight seal with the mouth or lip of a container such as a glass bottle, (3) overcoming objectionable irregularities in the liner surface and the container surface which might produce leakage, (4) eliminating in many instances the necessity of a center spot facing, and (5) offsetting any deficiency of the cellulosic cushion liner in resiliency and compressibility.

The foregoing advantages of the invention have been established by severe tests of crowns provided with sealing film coated liners in which cases of carbonated goods were inverted, then rolled over several times one way and then in the reverse direction, then dropped 9" and finally stored for several weeks. At the end of the tests, all of the bottles showed from 3.48 to 3.53 volumes of gas which was just a little higher than that with the composition cork control liners.

A further object of the invention is to provide a cap having a cushion liner provided with a sealing film which is thoroughly sanitary and non-toxic, and which moreover gives a nice appearance to the cap, both before application to and after removal from the container.

An additional object of the invention is to provide a cap having a cellulosic cushion liner coated with a sealing film which is sufficiently thermoplastic to permit the application of a center spot without the necessity of employing an independent adhesive to adhere the spot to the cushion liner.

Of equal importance with the foregoing is an object of the invention to provide cushion lining material which may be readily prepared from a compressed or densified cellulosic body, such a pulp board, board composed of wood fibers and cotton fibers, as well as gray cotton board, by dipping strips of suitable thickness into the sealing film solution and forming on the surface of the board a sealing film of the desired depth. As explained, this sealing film is deposited from solution and on drying in the air, or by forced drying, or by accelerated drying with heat, a thermoplastic coating is produced which is stable and thoroughly reliable. The cushion liners may be punched from such a board or strip of board material, and since both sides of the liner will be provided with an adherent sealing film of uniform desired thickness, no care is needed in

2

stacking the disks for use in the liner inserting machines, as distinguished from operations where a single surface only of the cushion liner is provided with a protective coating. The present invention provides a very acceptable substitute for the usual cork composition liners, and also meets the demand for an inexpensive article which is reversible, i. e. can be fed into the hopper of the automatic cap assembling machine without the necessity of being stacked right side up.

In carrying out the invention, cellulosic board of the character above mentioned composed wholly of wood fibers as described in the copending application of Warth, Serial No. 401,852, now abandoned, or the copending application of Costa and Ryan, Serial No. 418,248 now Patent No. 2,338,705 is preferred, but any suitable cellulosic board may be used since the sealing film of the present invention overcomes effectively any deficiencies in resiliency or compressibility between the board and the usual cork composition. Preferably, the cushion board is approximately .050" in thickness, and is provided with a sealing film by running the board as an endless band or strip through a bath of the prepared coating material at a slow speed so that the material drains back to prevent any objectionable film characteristics from developing on the board. The coating is thus applied to both sides of the board. In the case of a coating for a spot crown, the thickness of the coating is about .0025" for each side. As explained above, it is unnecessary to use a center spot with cushion liners in accordance with the present invention since a coating of approximately .005" for each side may be readily obtained, or even greater thicknesses by subjecting the board to a suitable treatment, such as one or more dippings until the desired thickness of coating is built up. The thickness of the film takes up the inequalities or roughness in the surface of the board. We have found that even so-called "smooth boards" do have inequalities or rough spots on the surface which are eliminated by the sealing film.

The drying of the coated board is accomplished with a low degree of heat, e. g. about 150° F. to 200° F., the temperature depending upon the height of the drying tower, which is preferably used. The coating, however, can be dried at room temperature, or by forced drying.

It will be appreciated that by simply running the cushion board through an inexpensive coating material, the product obtained is much less costly than treating the cushion board with a facing of "Vinylite" resin or other paper facings, such as gloss papers, particularly where such resins or papers are applied to both sides of the board.

Instead of a dipping procedure, the board may

be coated on an intaglio coating machine which applies the coating material by means of wire wound rods serving to brush the coating on the board in a uniform manner. The board is passed through a tunnel drier whence it goes on a rewinding roll in the dry condition.

The sealing film preferably comprises resin, a wax, and clay in finely divided state. In some cases, the clay may be omitted. The resin is in greater amount than the wax, while the clay is in greater amount than either the resin or wax. The material is dissolved or suspended in a suitable solvent which is evaporated off in the drying, and the dried and coated board is then rewound.

A preferred example employing resin, wax and clay is here illustrated:

*Example A*

|                  | Parts by weight |
|------------------|-----------------|
| Resin            | 18.75           |
| Wax              | 2.50            |
| Clay             | 22.50           |
| <br>Total solids | 43.75           |
| #2220 solvent    | 56.25           |

The resin used is N-butyl methacrylate resin. The wax is pale yellow amorphoid wax 180° F. melting point, also referred to as a well refined petroleum wax. The clay is a kaolin clay of about 300 mesh fineness. A very fine mesh is needed to keep the clay in suspension in the finished coating. The solvent is an aromatic hydrocarbon solvent made by the Shell Oil Company.

The clay is thoroughly dispersed in the resin and wax by means of a ball mill. This grinding takes a number of hours and is preferred to the colloidal mill since larger batches can be handled with relatively little labor. The solution or suspension will contain 43.75% of non-volatile solids and 56.25% of solvent.

Another preferred example illustrating a modification of proportions is the following:

*Example B*

|                            | Grams |
|----------------------------|-------|
| N-butyl methacrylate resin | 75    |
| 180 pale yellow wax        | 10    |
| 2220 solvent (Shell)       | 225   |
| Clay (Dixie)               | 90    |

The wax is used for the purpose of increasing the melting point and providing a smoother finish as distinguished from a coating which lacks wax and which has a somewhat crystalline surface appearance.

Any high melting point amorphoid or petroleum hydrocarbon wax can be used in place of the pale yellow wax, e. g., a white amorphoid wax of 170° F. melting point.

The solvent, of which many are commercially available, is essentially an aromatic hydrocarbon solvent, having an initial boiling point of not less than 145° F., and a dry point of not more than 300° F., with the flash point below 40° F.

In order to secure greater flexibility of the coating, suitable plasticizers may be added to the ingredients in the formulas, e. g., stearic acid.

In the accompanying drawing, we have illustrated the invention as applied to a crown cap, but it is to be understood as set forth above, that it is applicable to all forms of caps in which a cushion liner is utilized.

Referring to the drawings,

Figure 1 is a section of a crown cap having a cushion liner assembled therein in accordance with this invention:

Figure 2 is a sectional view of the coated board; and

Figure 3 is a view similar to Figure 1 in which the cushion liner is provided with a center facing spot.

The cap of Figure 1 comprises a metal shell 10 having a skirt 11 provided with the usual crimps 12. The cushion liner is indicated at 13 as a whole and includes the cellulosic board layer 14 and films 15 and 16 of one of the materials described above. As stated, these films are deposited from a solution and are firmly adhered to one or both faces of the cellulosic layer 14. In Figure 2 there is shown the coated board from which liners illustrated in Figures 1 and 3 are punched and assembled in the caps. Referring to Figure 3, there is employed a center spot 17 which is adhered to the sealing film layer 15 without the need of an independent adhesive. The thermoplasticity of the film 15 serves to tightly unite the spot to the film. It is not usually necessary to employ a center spot, but in some cases this may be desirable. The center spot may be of the customary paper, foil or chemical composition film material.

We claim:

1. A closure having a cushion liner therein of cellulosic material coated on at least one side with a coextensive, thermoplastic sealing film of N-butyl methacrylate resin, amorphoid wax and finely divided clay, the resin being present in greater amount than the wax and the clay being present in greater amount than the wax or resin.
2. A cushion liner for closures of cellulosic material coated on at least one side with a coextensive, thermoplastic sealing film of N-butyl methacrylate resin, amorphoid wax and finely divided clay, the resin being present in greater amount than the wax and the clay being present in greater amount than the wax or resin.

ALBIN H. WARTH.  
PAUL GRABUS, JR.

REFERENCES CITED

The following references are of record in the file of this patent:

UNITED STATES PATENTS

| Number    | Name            | Date          |
|-----------|-----------------|---------------|
| 748,586   | Coddington      | Jan. 5, 1904  |
| 983,319   | Smith et al.    | Feb. 5, 1911  |
| 1,123,206 | Gaston          | Dec. 29, 1914 |
| 1,144,589 | Fay             | June 29, 1915 |
| 1,215,737 | Stahl           | Feb. 13, 1917 |
| 1,609,562 | Lonsdale et al. | Dec. 7, 1926  |
| 1,656,514 | Wirth           | Jan. 17, 1928 |
| 1,804,555 | Gentile         | May 12, 1931  |
| 1,950,436 | Williams        | Mar. 13, 1934 |
| 2,067,066 | Schmidt et al.  | Jan. 5, 1937  |
| 2,073,415 | Enkur           | Mar. 9, 1937  |
| 2,091,180 | Magill          | Aug. 24, 1937 |
| 2,097,754 | Bradshaw        | Nov. 2, 1937  |
| 2,109,944 | Larson          | Mar. 1, 1938  |
| 2,181,481 | Gray            | Nov. 28, 1939 |
| 2,227,516 | Soanes          | Jan. 7, 1941  |
| 2,232,595 | Dittmar et al.  | Feb. 18, 1941 |
| 2,275,063 | Moore           | Mar. 3, 1942  |
| 2,290,392 | Thomas          | July 21, 1942 |
| 2,316,274 | Mitchell        | Apr. 13, 1943 |
| 2,338,705 | Costa et al.    | Jan. 11, 1944 |
| 2,341,925 | Kulman          | Feb. 15, 1944 |